

1

3,188,163

BLUE DYED POLYPROPYLENE FIBERS AND  
PROCESS OF DYEING THEM

Joseph W. Dehn, Jr., Great Neck, and Harold J. Kuhefuss, Brooklyn, N.Y., assignors to Interchemical Corporation, New York, N.Y., a corporation of Ohio  
No Drawing. Filed Jan. 22, 1963, Ser. No. 253,041  
2 Claims. (Cl. 8—39)

This invention relates to blue dyed polypropylene fibers and textiles and to a process for dyeing them.

We have found that textiles composed of polypropylene fibers may be dyed blue with good strength and build-up, using a more or less conventional method for disperse dyeing, with 1,4-bis-(2',4',6'-triethylanilino)-anthraquinone. The blue textiles display superior washfastness and lightfastness, and the dye has better affinity for the fiber than do the commercially available blue dyes now recommended for such dyeings. The compound is one known to the art, but the art had hitherto no knowledge of its value or even of its possible use as a polypropylene dye.

The dyeing is conveniently carried out by dispersing 1,4-bis-(2',4',6'-triethylanilino)-anthraquinone with suitable dispersing agents and immersing the polypropylene textile in the dyebath, heated to around boiling temperature, for an hour or two.

The dyed fibers of this invention were evaluated along with dyeings similarly made with the best available commercial blue dyestuffs recommended by the manufacturer of the polypropylene fibers used in these tests. Fibers dyed according to this invention showed definite superiority over those dyed according to the manufacturer's recommendations, in washfastness, lightfastness, and affinity of the dye for the fiber.

## Example 1

A mixture of 2.00 g. of 1,4-bis-(2',4',6'-triethylanilino)-anthraquinone (a commercially available chemical), 1.00 g. of Marasperse N, and 1.00 g. of Cyclopon AF was ground with a hand muller in the presence of water. The resulting dispersion was dried in an oven at about 50° C. and the dried material was ground to a powder with mortar and pestle. This material was used in a dyebath. Polypropylene cloth of convenient size was scoured 30 minutes at 70° C. in a bath containing an anionic wetting agent, such as Sulframin AB to the amount of about 1% by weight based on the weight of the cloth and 0.25% by weight (same basis) of sodium carbonate.

A dyebath was made up, the total amount being about 40 times the weight of the cloth to be dyed. The bath contained 1%, based on the weight of cloth, of Sulframin AB and 1/2% of dye on the same basis. The goods were entered at room temperature and the bath heated to boiling for about 2 hours. To remove surface dye the goods were then soaped 30 minutes at 70° C. in a solution similar to the scouring bath, the difference being that instead of 0.25% sodium carbonate, this bath had 2%.

## Example 2

Similarly dyeings were made using 2% of dye based on the weight of cloth. Both 1/2% and 2% dyeings were used in the evaluation tests.

Instead of sodium carbonate in the scouring bath other suitable alkalies may be used, the pH of such baths being in the neighborhood of 11-12.

## Example 3

50 mg. of dye dispersion was made into a paste with 5 cc. of a 1% aqueous Triton X-100 solution and the

2

paste diluted with 295 cc. of water. 10 g. of polypropylene cloth was entered in the bath, which was then heated on the steam bath at a temperature of 200° F. for 45 minutes. The cloth was then removed and the dyebath restored to its original volume with warm water. The pH was adjusted to 3.5-4 with formic acid. The cloth was replaced in the bath and dyed at 200° F. for 30 minutes more. A soaping with Duponol RA, a rinse with water, and air drying completed the process.

## Example 4

The foregoing process was repeated using 200 mg. of dye dispersion instead of 50 mg., thus yielding a 2.0% dyeing instead of a 1/2% dyeing.

The dispersing agent used is not critical; any reasonably efficient one will do. A few suitable are here listed by way of example. "Marasperse N" (sodium ligno sulfate); "Marasperse CB" (partially desulfonated sodium ligno sulfate); "Blancol N" (sodium salt of a sulfonated naphthalene and formaldehyde condensate); "Tanol SN" (a neutral salt of a complex condensed aryl organic acid); "Cyclopon AF" (sodium N-acyl-N-methyl taurate); "Igepon CN-42" (sodium N-cyclohexyl-N-palmitoyl taurate); "Igepons T-33, T-43, T-51, T-73, T-77" (sodium N-methyl-N-oleyl taurates); "Igepon TE-42" (sodium N-methyl-N-tallow acid taurate); "Igepon TN-54" (sodium N-methyl-N-palmitoyl taurate).

Many anionic and non-ionic surfactants are suitable. No critical limitation appears to exist. As examples of suitable surfactants there may be mentioned "Sulframin AB" (sodium alkyl benzene sulfonate); "Nacconol NR" (sodium alkylaryl); "Duponol ME" (a long chain alcohol sulfate sodium salt); "Tergitol NP-9" or "Tergitol NP-40" (nonylphenyl polyethylene glycol ether); "Tergitol NP-14" (or NP-27 or NP-35 or TMN) (other alkylaryl polyglycols); "Triton X-100" (other alkylaryl polyether glycols which are reaction products of tertiary-octyl phenol with ethylene oxide). "Duponol RA" is a fortified ether-alcohol sulfate.

What is claimed is:

1. Blue-dyed polypropylene fibers, the dye being 1,4-bis-(2',4',6'-triethylanilino) anthraquinone.
2. Process for dyeing polypropylene fibers blue, consisting essentially of
  - (a) immersing polypropylene fiber in an aqueous dyebath containing conventional amounts of the dye, 1,4-bis(2',4',6'-triethyl anilino) anthraquinone dispersed therein and a suitable dispersing agent,
  - (b) heating the bath to around 200° F. for about 1-2 hours,
  - (c) removing the fiber from the bath and drying.

## References Cited by the Examiner

## UNITED STATES PATENTS

|           |       |                        |           |
|-----------|-------|------------------------|-----------|
| 2,051,004 | 8/36  | Koerberle et al. ----- | 260—378   |
| 2,131,098 | 9/38  | Dreyfus -----          | 8—55      |
| 2,152,191 | 3/39  | Herrett -----          | 260—378   |
| 2,596,820 | 5/52  | Ogilvie -----          | 260—378 X |
| 2,605,269 | 7/52  | Buxbaum -----          | 260—378 X |
| 2,736,731 | 2/56  | Peter et al. -----     | 260—378 X |
| 2,893,985 | 7/59  | Powelson -----         | 260—94.9  |
| 3,052,510 | 9/62  | Simpson et al. -----   | 8—55      |
| 3,059,987 | 10/62 | Bauman -----           | 8—55      |

## FOREIGN PATENTS

494,802 11/38 Great Britain.

70 NORMAN G. TORCHIN, Primary Examiner.  
ABRAHAM H. WINKELSTEIN, Examiner.